



US007201642B2

(12) **United States Patent**  
**Koh et al.**

(10) **Patent No.:** **US 7,201,642 B2**  
(45) **Date of Patent:** **Apr. 10, 2007**

(54) **PROCESS FOR PRODUCING IMPROVED MEMBRANES**

(75) Inventors: **Meng Fei Koh**, Singapore (SG); **Choon Siong Poh**, Singapore (SG); **Inn Swee Goh**, Singapore (SG); **Theng Wei Leong**, Singapore (SG); **Teck Leong Neo**, Singapore (SG); **Bing Wang**, Singapore (SG)

(73) Assignee: **Systems on Silicon Manufacturing Co. Pte. Ltd.**, Singapore (SG)

(\*) Notice: Subject to any disclaimer, the term of this patent is extended or adjusted under 35 U.S.C. 154(b) by 0 days.

(21) Appl. No.: **10/544,010**

(22) PCT Filed: **Jun. 14, 2004**

(86) PCT No.: **PCT/SG2004/000183**

§ 371 (c)(1),  
(2), (4) Date: **Aug. 1, 2005**

(87) PCT Pub. No.: **WO2005/123342**

PCT Pub. Date: **Dec. 29, 2005**

(65) **Prior Publication Data**

US 2006/0258273 A1 Nov. 16, 2006

(51) **Int. Cl.**  
**B24B 1/00** (2006.01)

(52) **U.S. Cl.** ..... **451/53; 451/7**

(58) **Field of Classification Search** ..... **451/7, 451/53, 285-289, 388, 397, 398**  
See application file for complete search history.

(56) **References Cited**

**U.S. PATENT DOCUMENTS**

|                |        |               |        |
|----------------|--------|---------------|--------|
| 6,077,151 A *  | 6/2000 | Black et al.  | 451/53 |
| 6,080,050 A    | 6/2000 | Chen et al.   |        |
| 6,183,354 B1   | 2/2001 | Zuniga et al. |        |
| 6,506,104 B2   | 1/2003 | Perlov et al. |        |
| 6,540,594 B2   | 4/2003 | Zuniga et al. |        |
| 6,602,114 B1 * | 8/2003 | Wang et al.   | 451/41 |
| 6,705,923 B2 * | 3/2004 | Liu et al.    | 451/7  |
| 6,705,924 B2 * | 3/2004 | Somekh        | 451/9  |

**FOREIGN PATENT DOCUMENTS**

|    |               |         |
|----|---------------|---------|
| JP | 2003 142438 A | 5/2003  |
| JP | 2003 297784 A | 10/2003 |

\* cited by examiner

*Primary Examiner*—Dung Van Nguyen

(74) *Attorney, Agent, or Firm*—Harness, Dickey & Pierce, P.L.C.

(57) **ABSTRACT**

The present invention relates generally to the field of chemical/mechanical polishing of substrates. In particular the invention relates to methods of producing improved membranes for use in chemical/mechanical polishing systems. The present invention provides a method of improving the properties of a flexible membrane for use in chemical/mechanical polishing, the method including subjecting the membrane to elevated temperatures.

**13 Claims, 3 Drawing Sheets**



Fig 1





Fig 2

Fig 3

## Weekly slips per 10k W+ Mirra moves



## 1

PROCESS FOR PRODUCING IMPROVED  
MEMBRANES

## FIELD OF THE INVENTION

The present invention relates generally to the field of chemical/mechanical polishing of substrates. In particular the invention relates to methods of producing improved membranes for use in chemical/mechanical polishing systems.

## BACKGROUND OF THE INVENTION

With the rapid development of the electronics industry in recent years there has been phenomenal growth in the need for integrated circuits. As such there has been a significant focus world-wide on improving methods of manufacture of integrated circuits with a view to increasing production speed/efficiency. In general integrated circuits may be formed on a number of materials but they are typically formed on silicon wafers. The process of manufacture of integrated circuits of this type typically involves the sequential deposition of a number of layers of conductive, semi-conductive or insulating layers onto the outer surface of a wafer. Using the process a number of layers are built up sequentially with each deposited layer becoming the new outer surface of the wafer. The wafer thus formed is typically etched after each layer is deposited so as to form the desired final circuitry features of the integrated circuit onto the wafer. As successive etched layers are built up the final form of the integrated circuit is produced.

One problem that potentially occurs in this process is that as the sequential layers are deposited and etched in this way, the outer surface becomes increasingly non-planar. This in turn causes difficulty as if the outer surface is non-planar then, as a consequence, any further layers placed on the outer layer will also be non-planar. As this reduces the performance of the final integrated circuit a number of approaches have been developed in order to produce planar surfaces as the successive layers are set down.

Chemical/mechanical polishing (CMP) is one of the preferred methods of planarization of substrate surfaces which has been used to alleviate this problem and which has found use in the manufacture of integrated circuits. This method typically requires mounting the substrate (such as the wafer) onto a carrier or polishing head in some way. The exposed surface of the substrate is then placed against a rotating polishing pad which removes excess material from the uneven topography on the surface of the substrate until a substantially flat (planar) surface has been created. The carrier head typically is configured to provide a controllable load pressure onto the substrate to press it evenly against the polishing pad to ensure even polishing across the surface of the substrate. A number of different carrier heads and/or polishing systems have been developed for use in chemical/mechanical polishing processes of this type.

A problem identified in the development of the carrier heads of this type has been the need to design a head that does not damage sensitive substrates such as the silicon wafers during handling. Silicon wafers that are subjected to the process are generally very thin and hence are not ideally suited to being brought into contact with any hard surfaces during movement operations. In addition, even if the surface of the head can be padded in some way there is the risk that the point of contact with the wafer may cause the surface of the wafer to become marked. In order to overcome these difficulties a number of techniques have been used. One

## 2

technique that has found general application has been the use of flexible membranes that contact the substrate (wafer). In use these are actuated by creating a vacuum behind the membrane forming "suction cups" that contact the wafer and provide a "chucking" effect such that the wafer is held on the membrane. This has been found to effectively hold the wafers so that they can be moved by the head without causing the problems discussed above. In addition by pressurising a chamber behind the membrane, the membrane can force the wafer onto a polishing pad and assist in the polishing process. Accordingly there are a large number of carrier heads that contain flexible membranes in one configuration or another.

For example one suitable carrier head of this type is described in U.S. Pat. No. 6,080,050. This describes a carrier head including a flexible membrane and a compliant backing member for a chemical/mechanical polishing apparatus. The carrier head includes a flexible membrane, the lower surface of which provides a substrate receiving surface. The carrier head includes a compliant backing member with a plurality of cells which contact an upper surface of the flexible membrane to improve vacuum chucking of the substrate onto the head.

In another system, described in U.S. Pat. No. 6,183,354 there is described a carrier head for a chemical/mechanical polishing apparatus which includes a flexible membrane. The carrier head comprises a base, a support structure connected to the base by a flexure, and a flexible membrane connected to the support structure. The flexible membrane has a mounting surface for a substrate and extends beneath the support structure to define a chamber. The chamber may either be evacuated to form suction cups that grip the wafer when it is being moved or be pressurized in order to force the wafer onto the polishing surface during the polishing operation.

In yet another patent, namely U.S. Pat. No. 6,540,594 there is described a carrier head for a chemical/mechanical polishing apparatus comprising a base, a flexible membrane, and a retaining ring surrounding the central portion of the flexible membrane. The flexible membrane has a central portion with a mounting surface for a substrate and a perimeter portion connected to the base, the membrane extending beneath the base to define a chamber. The apparatus also includes a retaining ring surrounding the centre portion of the flexible membrane so as to hold the substrate in position especially when the membrane is pressurized.

Another carrier head that includes a flexible membrane is described in U.S. Pat. No. 6,506,104. This patent describes a carrier head with a flexible member connected to a base to define a first chamber, a second chamber and a third chamber. A lower surface of the flexible member provides a substrate receiving surface with an inner portion associated with the first chamber, a substantially annular middle portion surrounding the inner portion and associated with the second chamber, and a substantially annular portion surrounding the middle portion and associated with the third chamber. The use of a plurality of chambers allows for differential pressure to be applied by the head to different portions of the membrane and hence to the wafer.

As can be seen, there are a number of carrier heads that have been developed which all include flexible membranes in their construction. Indeed the carrier heads described above represent a mere subset of the number of heads that have been described which incorporate a flexible membrane.

One problem typically encountered with the use of a flexible membranes in carrier heads of these types is membrane failure whilst in use. The failure of the membrane

cannot be accurately predicted by conventional test procedures which do not damage the membrane. Accordingly it is not possible to test individual membranes prior to use and as such membrane failure typically occurs when in use. With existing membranes the failure rate is approximately 3.5 failures per 10,000 wafer moves. This leads to significant downtime consequences as membrane failure typically leads to the wafer being dropped in the chemical/mechanical polishing apparatus. Whenever this happens it is necessary to rebuild the heads including application of a new membrane, replacement of any damaged tool parts and consumables and recovery of dropped wafers. Due to the high cleanliness required there is also the risk that there may be contamination of the apparatus by any broken pieces of wafer that have occurred due to wafer damage upon falling. Typically, it is found that whenever a wafer drop occurs it takes something of the order of 2 hours to rebuild the head and 4-6 hours to place the apparatus back in full manufacturing mode. As will be appreciated, this leads to significant machine downtime and reduction in the overall sufficiency of the manufacturing process. Accordingly there is a need to develop improved membranes for use in apparatus of this type in order to reduce this downtime. Any reduction in the incidence of membrane failure will directly lead to improved manufacturing efficiencies for machines of this type.

In order to attempt to overcome this problem the current applicants studied membranes and membrane properties at some length in relation to the conditions under which these membranes were forced to operate. It was found that the poor membrane performance typically occurred due to poor selection of physical properties of the membranes used in that the membranes used did not have physical properties that were compatible with the conditions they were required to operate under. Accordingly, there was an unacceptably high rate of failure of the existing membranes during use.

As a result of their studies the applicants have found that functional ability of the membrane was affected by a number of interacting physical parameters. Without wishing to be bound by theory it is felt that insufficient membrane performance is observed when one or more of the membrane's physical properties is not within the required bounds. Unfortunately, the ability to test these physical parameters relies on destructive means and, as such, it is not possible to accurately predict the performance of an individual membrane prior to use by testing its physical parameters.

#### SUMMARY OF THE INVENTION

The applicants of the present application were able to ascertain that significantly improved membrane performance in carrier heads could be achieved by treating the membranes either during membrane manufacture or as a step prior to using the membrane. In particular the applicants found that subjecting the current membranes to elevated temperatures improved the performance characteristics of the membranes.

The applicants have been successful in identifying process conditions that may be applied to existing membranes so that they have improved performance relative to untreated membranes. This allows existing membranes that can be purchased commercially to be converted into membranes with improved performance.

In one aspect the present invention provides a method of improving the performance of a flexible membrane for use in a chemical mechanical polishing system, the method including subjecting the flexible membrane to elevated temperatures.

The flexible membrane can be made of any suitable material typically used in membranes for chemical/mechanical polishing however the preferred membrane includes silicone rubber.

5 The flexible membrane may be of any suitable size for use in a chemical mechanical polishing system and the physical dimensions will typically be determined from the size of the carrier head. Nevertheless the membranes subjected to the process typically have a thickness of from 0.2 to 1.4 mm, 10 more preferably from 0.6 to 1.0 mm, most preferably about 0.8 mm.

The flexible membrane may be subjected to the elevated temperature for a wide range of time periods with the time period being determined by the elevated temperature. The 15 period of time may be any period that achieves the desired result however it is preferred that the period is no more than 24 hours, although longer treatment times have been found to work. The treatment period is typically from 5 minutes to 24 hours, more preferably from 5 minutes to 240 minutes, 20 even more preferably from 10 minutes to 180 minutes, yet even more preferably from 20 minutes to 120 minutes, most preferably from 30 minutes to 90 minutes. The elevated temperature of the treatment is typically from 50° C. to 150° C., more preferably from 50° C. to 100° C., even more preferably from 60° C. to 95° C., most preferably from 75° C. to 90° C.

As will be readily appreciated there is a relationship between the duration of the treatment period and the temperature of the treatment. Typically it is found that the higher 30 the temperature the shorter treatment time required. It is preferred that the treatment involves subjecting the flexible membrane to a temperature of from 50° C. to 100° C. for a period of from 15 minutes to 120 minutes. It is even more preferred that the flexible membrane is subjected to a temperature of from 60° C. to 95° C. for a period of from 30 minutes to 90 minutes. In a most preferred embodiment the membrane is subjected to a temperature of from 75° C. to 90° C. for a period of from 30 minutes to 90 minutes, most preferably from 60 minutes to 90 minutes. A number of 40 specific regimes within these ranges are particularly preferred. One preferred regime is 90° C. for 60 minutes. Another preferred regime is 80° C. for 60 minutes. A further preferred regime is 75° C. for 120 minutes.

The membranes subjected to the process may be of any 45 suitable type. Particularly preferred membranes include silicone rubber, preferably high strength silicone rubber.

It has been found that by using membranes that have been subjected to a process of this type membrane failure during the chemical/mechanical polishing of wafers is significantly 50 lowered. This in turn leads to significantly reduced machine downtime as the heads have to be rebuilt far less frequently and the number of dropped wafers is also significantly reduced. This therefore leads to considerably higher manufacturing efficiency.

55 As stated previously the membranes that have been subjected to the process may be used in any carrier head for chemical/mechanical polishing that includes a flexible membrane. When the membranes treated by the process are utilised in carrier heads of this type the carrier heads 60 typically demonstrate improved performance due to lower levels of membrane failure.

In another embodiment the present invention provides a carrier head for a chemical/mechanical polishing apparatus. The carrier head includes a base and a flexible membrane, 65 the flexible membrane has a mounting surface for a substrate and extends beneath the base to define a boundary of a pressurizable chamber, the flexible membrane having been

subjected to the process of the invention. The membrane preferably has a maximum tensile strength of at least 10.5 MPa, more preferably a tensile strength of at least 11.0 MPa. The membrane also preferably has an elongation at break of at least 820%, more preferably 850%. It is preferred that the flexible membrane has a central portion forming a mounting surface for a substrate and a peripheral portion that is preferably in contact with the base, the membrane extending beneath the base to define a chamber.

The carrier head preferably also includes a retaining ring which surrounds the central portion of the membrane. In a further preferred embodiment the retaining ring is connected to the base.

The carrier head also preferably further includes a support structure that is movable relative to the base, the support structure being located between the base and the flexible membrane. In a particularly preferred embodiment the peripheral portion of the flexible membrane is attached to the support structure, preferably extending around an edge of the support structure. In a further preferred embodiment the carrier head further includes a flexure connecting the support structure to the base. Preferably the flexure undergoes bending to allow the support structure and the flexible membrane to move away from the base as fluid is forced into the chamber.

In one preferred embodiment the support structure includes an annular ring and the membrane preferably extends around an outer rim of the annular ring. In this embodiment it is preferred that the chamber includes a first portion located above the annular ring and a second portion located below the annular ring.

In another preferred embodiment the support structure includes a circular plate. In this embodiment it is preferred that the chamber includes a first portion located above the annular ring and a second portion located below the annular ring.

In a preferred embodiment the support structure has at least one aperture therethrough to connect a first portion of the chamber between the flexible membrane and the support structure to a second portion of the chamber between the support structure and the base. In this embodiment the flexible membrane and support structure moves away from the base when fluid is forced into the chamber. It is preferred in this embodiment that the support structure contacts the surface of the flexible membrane. In a particularly preferred embodiment the support structure includes a plurality of apertures.

#### BRIEF DESCRIPTION OF THE FIGURES

FIG. 1 This shows a sectional view of a carrier head incorporating a membrane.

FIG. 2 This shows a sectional view of a portion of the carrier head of FIG. 1 following membrane failure.

FIG. 3 This shows a graph demonstrating the results of an extended trial in which a pilot plant was operated with commercially available membranes followed by replacement of these membranes with membranes treated by the process of the invention.

#### DETAILED DESCRIPTION OF THE INVENTION

The present invention provides improved membranes for use in chemical/mechanical polishing systems. In chemical mechanical polishing systems flexible membranes are used extensively and the way in which they are used is shown for

example in FIG. 1. With reference to FIG. 1 there is shown a carrier head with an upper assembly (1) and a retaining ring (2). The carrier head includes a perforated support structure (3) which is located within the retaining ring (2). A flexible membrane (4) sits on the support structure and when a vacuum is applied the membrane (4) extends through apertures in the support structure (3) forming a plurality of suction cups (5). These suction cups hold onto wafer (6) such that it is held onto the carrier head by vacuum.

10 The problem that occurs with membranes of this type is shown in FIG. 2 which depicts an exploded view of the carrier head of FIG. 1. If the membrane (4) fails the suction cups collapse and this releases the vacuum holding the wafer onto the membrane. When this occurs the wafer drops. There 15 is therefore a need to develop improved membranes for use in CMP systems.

The applicants have found that the membranes to be subjected to the process of the invention can be manufactured de novo using well established membrane fabrication 20 techniques. Accordingly the membranes to be subjected to the process may be purchased commercially. It has been found, however, that one of the simplest modifications of the known procedures is the incorporation of an additional treatment step into the production process for these membranes. This additional treatment step can be carried out at the end of the existing production process prior to the packaging of the known membranes, or alternatively, the existing packaged membranes may be subjected to the additional processing step at a later stage. For example the 25 membranes may be subjected to the additional processing step just prior to use at the integrated circuit plant. One advantage of conducting the additional processing just prior to use is that it ensures no deterioration of the membrane properties before use.

30 The present invention therefore provides a method of improving the performance of a flexible membrane for use in a chemical/mechanical polishing system, the method including subjecting the membrane to elevated temperatures. It is preferred that following the treatment the membrane 35 has a maximum tensile strength of at least 10 MPa and an elongation at break of at least 800%. It is further preferred that the membrane is treated until it has a maximum tensile strength of at least 10.5 MPa, more preferably at least 11.0 MPa. It is also preferred that the treatment is such that the 40 membrane following treatment has an elongation at break of at least 820%, more preferably at least 850%.

The treatment period may be of any suitable time but is 45 preferably no longer than 24 hours. The treatment period is typically from 5 minutes to 24 hours, more preferably from 5 minutes to 240 minutes, even more preferably from 10 minutes to 180 minutes, yet even more preferably from 20 minutes to 120 minutes, more preferably from 30 minutes to 90 minutes, most preferably from 60 to 90 minutes. The elevated temperature of the treatment is typically from 50° C. to 150° C., more preferably from 50° C. to 100° C., even 50 more preferably from 60° C. to 95° C., most preferably from 75° C. to 90° C.

60 As will be readily appreciated there is a relationship between the duration of the treatment period and the temperature. Typically it is found that the higher the temperature the shorter time required. It is preferred that the treatment involves subjecting the membrane to a temperature of from 50° C. to 100° C. for a period of from 15 minutes to 120 minutes. It is even more preferred that the flexible membrane is subjected to a temperature of from 60° C. to 95° C. for a period of from 30 minutes to 90 minutes. In a most preferred embodiment the membrane is subjected to a tem-

perature of from 75° C. to 90° C. for a period of from 30 minutes to 90 minutes, most preferably from 60 minutes to 90 minutes. A number of specific regimes within these ranges are particularly preferred. One preferred regime is 90° C. for 60 minutes. Another preferred regime is 80° C. for 60 minutes. A further preferred regime is 75° C. for 120 minutes.

The heat treatment discussed above may be carried out in any suitable heating apparatus which does not introduce contaminants onto the surface of the membrane. Examples of suitable heating apparatus include heating ovens and chambers. Due to the need to reduce contamination it is preferred that the heat source is such that external heating of the oven chamber is carried out so that no residue of the heating enters the chamber. As such heating devices such as ovens including a "naked" gas flame are typically not preferred.

The heating may occur in a continuous fashion in which membranes are passed through a heated oven or chamber with the speed of passage being such as to hold the membrane in the chamber or oven for the required residence time. Column heating devices suitable for heating in this way are well known in which the membrane travels the length of the column and is heated in the column. Due to the length of the heating required, however, it is typical to heat the membranes in a batchwise fashion in which one or more (typically a large number) of membranes are placed in an oven at the required temperature and left to heat for the required time.

After the membrane has been heated it is removed from the heat source and preferably placed at ambient temperature and allowed to cool. This preferably occurs in a clean room environment with a temperature of between 20° C. to 23° C. and a relative humidity of about 50%. Alternatively the membrane may be rapidly cooled by being placed in a cooled chamber or by having a cooled fluid or gas passed over the membrane.

After treatment the membranes preferably have a maximum tensile strength of at least 10.5 MPa, more preferably at least 11 MPa. As used herein the maximum tensile strength of a membrane is determined using ASTM D638: 2000. Using this standard test procedure the tensile strength of the treated membranes were determined using the following parameters:

|                            |                         |
|----------------------------|-------------------------|
| Type of test species       | Dumb-bell Shape - Die C |
| Gauge Length               | 25 mm                   |
| Length of Grips Separating | 64 mm                   |
| Gross head speed           | 50 mm/min.              |

When reference to maximum tensile strength is referred to in the specification or claims it is measured using this test.

The elongation at break of the membrane after treatment is preferably at least 820%, more preferably at least 850%.

The flexible membrane may be of any suitable size that enables it to be used in carrier heads for chemical/mechanical polishing. As will be understood by a skilled addressee membranes used in chemical/mechanical polishing systems will vary depending on the size of the integrated circuit being produced and the dimensions of the carrier head that the membrane is intended to be used on. It has been found, however, that the improvements in membranes identified by the applicant are applicable irrespective of the size of the membrane required and thus is applicable to all membranes for chemical/mechanical polishing systems.

In addition the membrane can be any suitable shape to fit the configuration of the carrier head and shape of the integrated circuit being produced. Nevertheless the mem-

branes are typically substantially circular. Any suitable membrane thickness may suffice but it typically has a thickness of from 0.6 mm to 1.0 mm, most preferably a thickness of 0.8 mm.

The flexible membrane can be made of any suitable material typically used in membranes for chemical/mechanical polishing systems with the principle requirement that the membrane must be a flexible and elastic material. It is preferred that the membrane includes silicone rubber, preferably high strength silicone rubber.

The process may include a number of additional steps. For example the membrane may be washed prior to or after heating (or both) in order to remove any possible contaminants on the surface of the membrane. It is preferred that the membrane is washed with a solution to remove any organic contaminants on the surface. A suitable solution to achieve this is a solution of IPA (isopropyl alcohol) in water. The preferred concentration is 5% of IPA in water. It is also preferred that the membrane is washed with de-ionised water prior to treatment. It is found that such a washing step removes any residue left behind from other wash solutions (such as the IPA) and as well ensures that other particulate contaminants are removed.

The washing steps referred to above are carried out in ways well known in the art. It is preferred that the washing steps are carried out prior to treatment. If a washing step is included in the process the membrane is preferably dried prior to treatment. The drying may occur in any way known although it preferably involves air drying. Following completion of the treatment the membranes are stored prior to use.

The membranes that have been subjected to the process of the present invention may be used in any carrier head for a chemical/mechanical polishing system that incorporates at least one flexible membrane. Examples of preferred carrier head systems that may incorporate the flexible membranes treated by the process of the invention are those described in U.S. Pat. Nos. 6,080,050, 6,183,154, 6,540,594 and 6,506,104, the entire contents of which are herein incorporated by reference. As stated previously the use of the treated membranes significantly enhances carrier head life between failure.

In another embodiment the present invention therefore provides a carrier head for a chemical/mechanical polishing apparatus. The carrier head includes a base and a flexible membrane treated by the process of the invention, the flexible membrane has a mounting surface for a substrate and extends beneath the base to define a boundary of a pressurizable chamber. It is preferred that the flexible membrane has a central portion forming a mounting surface for a substrate and a peripheral portion that is preferably in contact with the base, the membrane extending beneath the base to define a chamber.

The carrier head preferably also includes a retaining ring which surrounds the central portion of the membrane. In a further preferred embodiment the retaining ring is connected to the base.

The retaining ring may be made of any suitable material. For example the retaining ring may preferably be made of a hard plastic or a similar material. The retaining ring may be secured to the carrier base in a number of ways well known in the art. It is preferred, however, that the retaining ring is secured to the carrier base by the use of bolts.

In general the retaining ring is secured at the outer edge of the carrier base. The retaining ring may be of any suitable shape and geometry for the carrier head used. Nevertheless the retaining ring is generally an annular ring with a substantially flat bottom surface.

In use, as the carrier head is lowered towards the polishing head of the chemical/mechanical polishing apparatus, a

portion of the retaining ring contacts the polishing pads. Once this occurs an inner surface of the retaining ring in combination with a bottom surface of the flexible membrane defines a substrate receiving recess. When in use in the polishing apparatus the retaining ring acts to ensure that the substrate stays in the substrate receiving recess so that the substrate is not removed from the recess during the polishing process.

The carrier head also preferably further includes a support structure that is movable relative to the base located between the base and the flexible membrane. In a particularly preferred embodiment the peripheral portion of the flexible membrane is attached to the support structure, preferably extending around an edge of the support structure. In a further preferred embodiment the carrier head further includes a flexure connecting the support structure to the base.

The flexure used may be of any suitable type defined in the art. It is found, however, that the flexure is a generally planar annular ring which is typically flexible in the vertical direction and may be flexible or rigid in the other direction. Any suitable flexures used in the art may be incorporated. However it is preferred that the material used to manufacture the flexure is chosen so that the flexure has a durometer measurement between 30 on the Shore A scale and 70 on the Shore D scale. Examples of materials that may be used to meet these physical characteristics include rubber such as neoprene, elastomeric coated fabrics such as NYLON or NOMEX, plastics, or composite materials such as fibre glass. In general, the amount of flexibility of the flexure can vary however it is typically found that the flexure should be such that it allows the support structure to move by approximately 0.2–0.3 mm. In a typical embodiment of the invention the outer edge of the flexure is secured between a lower surface of the base and an upper surface of the retaining ring discussed previously.

Preferably the flexure undergoes bending to allow the support structure and the flexible membrane to move away from the base as fluid is forced into the chamber.

The support structure may be made of any suitable hard material. In one preferred embodiment the support structure includes a generally annular ring. In this embodiment it is preferred that the pressurizable chamber includes a first portion located above the annular ring and a second portion located below the annular ring. It is preferred in this embodiment that the membrane extends around an outer rim of the annular ring.

In another embodiment the support structure includes a circular plate. In general the plate has a generally planar lower surface and is suspended in the chamber defined by the membrane by the flexure as discussed previously. It is preferred that the plate is located in the chamber such that the chamber includes a first portion located above the circular plate and a second portion located below the circular plate. It is particularly preferred that the circular plate includes at least one aperture to connect the first portion of the chamber to the second portion of the chamber. In a most preferred embodiment the circular plate includes a plurality of chambers.

A carrier head of the invention which incorporates a flexible membrane typically operates in the following fashion. A substrate is loaded onto the substrate receiving surface of the membrane with the back side of the substrate in contact with the mounting surface of the membrane. The pressurizable chamber is then expanded by fluid such as air being pumped into the chamber or, alternatively, the fluid is pumped into a bladder that is in contact with the chamber thus causing the chamber to be pressurized. This in turn places downward pressure on the membrane which is forced against the edge of the substrate creating a fluid-tight seal

between the substrate and the membrane. Once this has been achieved a pump is actuated to evacuate the chamber to create a low pressure pocket between the flexible membrane and the back side of the substrate thus chucking the substrate onto the membrane. As the substrate is then safely held onto the membrane the carrier head can then be actuated to move the membrane either to a transfer station or onto a polishing pad.

Of course, in embodiments where there are additional components in the carrier head these are involved in the process in ways well known in the art. As discussed previously there are a large number of other components that have been described for use in carrier heads, including flexible membranes which will not be discussed further.

The invention also relates to the use of the treated membranes of the invention as described above in a chemical/mechanical polishing system.

The present invention will now be described with reference to the following examples.

## EXAMPLE 1

In order to demonstrate the process of the invention a number of silicone membranes were subjected to the process of the invention. The silicone membranes were sourced from Applied Materials under Part Number 0021-77650. A group of 18 silicone membranes were subjected to varying temperature/time regimes and a number of physical properties were then measured. The regimes were:

1. Control—no treatment.
2. 50° C. for 60 minutes.
3. 70° C. for 60 minutes.
4. 80° C. for 60 minutes.
5. 90° C. for 60 minutes.

In each case the silicone membrane was removed from the packaging, wiped with a solution of 5% IPA in water to remove surface organic compounds. The surface was then wiped with de-ionized water to clean off any remaining surface residue. The membrane is then dried and heated at the required temperature for 60 minutes. At the end of the treatment the membrane is removed from the heat source and left to cool in a clean room environment (Class 100-100,000, 20-20° C., 50% relative humidity) for 60 minutes. The membrane is then re-wrapped. The membrane thus obtained was tested for maximum tensile strength (MPa), Shore A hardness, elongation at break % and modulus of elasticity. The results are shown in the following table.

| 50 | Sample     | S/No. | Silicone Membranes |                             |                         |                             |
|----|------------|-------|--------------------|-----------------------------|-------------------------|-----------------------------|
|    |            |       | Shore A Hardness   | Max. Tensile Strength (MPa) | Elongation at Break (%) | Modulus of Elasticity (MPa) |
| 55 | 1. Control | 1     | 75                 | 9.1                         | 717.5                   | 1.5                         |
|    |            | 2     | 75                 | 9.2                         | 713.7                   | 1.6                         |
| 60 | 2. 50° C.  | 1     | 76                 | 10.2                        | 831.9                   | 1.5                         |
|    |            | 2     | 77                 | 10.2                        | 843.1                   | 1.4                         |
|    |            | 3     | 77                 | 10.4                        | 839.1                   | 1.9                         |
|    |            | 4     | 75                 | 10.4                        | 805.6                   | 2.2                         |
| 65 | 3. 70° C.  | 1     | 77                 | 11.0                        | 824.5                   | 1.9                         |
|    |            | 2     | 77                 | 10.7                        | 809.2                   | 1.7                         |
|    |            | 3     | 78                 | 11.3                        | 890.9                   | 1.6                         |
|    |            | 4     | 79                 | 10.6                        | 760.2                   | 3.0                         |
| 65 | 4. 80° C.  | 1     | 75                 | 11.1                        | 860.3                   | 1.1                         |
|    |            | 2     | 74                 | 11.2                        | 827.4                   | 2.1                         |
|    |            | 3     | 75                 | 10.4                        | 807.3                   | 1.8                         |
|    |            | 4     | 74                 | 10.5                        | 817.5                   | 2.0                         |

-continued

| Silicone Membranes |       |                  |                             |                         |                             |
|--------------------|-------|------------------|-----------------------------|-------------------------|-----------------------------|
| Sample             | S/No. | Shore A Hardness | Max. Tensile Strength (MPa) | Elongation at Break (%) | Modulus of Elasticity (MPa) |
| 5. 90° C.          | 1     | 76               | 10.5                        | 863.6                   | 1.5                         |
|                    | 2     | 77               | 9.4                         | 805.7                   | 1.7                         |
|                    | 3     | 74               | 10.1                        | 867.5                   | 1.2                         |
|                    | 4     | 76               | 10.7                        | 852.6                   | 1.8                         |

As can be seen the prior art membranes with the unacceptable performance characteristics typically have a maximum tensile strength of less than 10 MPa on an elongation at break of the order of about 700%. As discussed previously membrane failure when membranes of this type are used is of the order of 3.5 wafer drops (membrane failures) per 10,000 wafer moves. In effect, this equals the membrane failing after it has been activated on average 3,000 times.

The treated membranes that have been subjected to the process of the invention, in contrast, typically have a maximum tensile strength of at least 10 MPa and an elongation at break of in excess of 800%. Whilst this change may seem small following the use of the treated membranes the membrane failure rate drops to as low as 1 wafer drop (membrane failure) per 10,000 wafer moves. This equates to the membrane being activated more than 10,000 times on average before it fails. This change therefore more than triples the effective membrane life.

## EXAMPLE 2

A number of silicon membranes were prepared according to the general method outlined in Example 1. These were then subjected to a wafer grip test.

This typically involves placing a membrane on the carrier head and inverting it on a test surface. A transport cover is slid over the head and the wafer grip test function is activated. The retaining ring is then pressurized and presses against the cover. This is followed by the membrane being pushed against the cover by pressure until it presses flat on the cover to make full contact. The membrane is then subjected to vacuum which creates small suction cups with the help of a perforated backing plate which grips the cover. In order to rate a pass the membrane must stick to the cover for at least 1 minute. If the membrane fails it collapses immediately when the vacuum is applied.

For each membrane the grip test was performed 10 times. The applicants have found that the results of the grip test correlate to membrane performance.

| Process Variables |                  |                |
|-------------------|------------------|----------------|
| Temperature       | Time of Exposure | Grip Test Pass |
| 50° C.            | 120 m            | 90             |
| 50° C.            | 60 m             | 80             |
| 75° C.            | 60 m             | 95             |
| 75° C.            | 120 m            | 100            |
| 80° C.            | 60 m             | 100            |
| 90° C.            | 60 m             | 100            |
| 100° C.           | 30 m             | 100            |

As can be seen treating the membranes at temperatures of from 75° C. to 100° C. gave the best grip test possible. With

5

reference to the 75° C. treatment it can be seen that with lower temperatures an extended treatment time of 120 minutes rather than 60 minutes improves wafer performance from 95% to 100%.

## EXAMPLE 3

As a result of the improvements demonstrated by the membranes treated by the process of the invention it was decided to take a batch membranes that had been subjected to the process of the invention. These were then trialled in a pilot scale laboratory under full factory operating condition. This was to enable to full number of wafer movements to be carried out to ensure that the date obtained was statistically significant. The results are shown as FIG. 3. As can be seen in FIG. 3 the prior art membrane had a rate of membrane failure such that there were 3.35 wafer slips per 10,000 membrane movements. Following replacement of the prior art membrane with membranes that had been treated thus reduced to 1.47 wafer slips per 10,000 movements. This demonstrates the efficacy of the process of the invention in improving flexible membrane performance.

10 25 The invention claimed is:

1. A method of improving the properties of a flexible membrane for use in chemical/mechanical polishing, the method including subjecting the membrane to elevated temperatures of from 50° C. to 150° C.

15 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 500 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 600 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 700 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 800 9005 9010 9015 9020 9025 9030 9035 9040 9045 9050 9055 9060 9065 9070 9075 9080 9085 9090 9095 9

UNITED STATES PATENT AND TRADEMARK OFFICE  
**CERTIFICATE OF CORRECTION**

PATENT NO. : 7,201,642 B2  
APPLICATION NO. : 10/544010  
DATED : April 10, 2007  
INVENTOR(S) : Meng Fei Koh et al.

Page 1 of 1

It is certified that error appears in the above-identified patent and that said Letters Patent is hereby corrected as shown below:

On title page  
Item [22] delete "Jun. 14, 2004" and insert therefore --**June 17, 2004**--.

Signed and Sealed this

Thirty-first Day of July, 2007

A handwritten signature in black ink, appearing to read "Jon W. Dudas", is centered within a rectangular box with a dotted background.

JON W. DUDAS  
*Director of the United States Patent and Trademark Office*